

# United States Patent [19]

Saito et al.

[11] 3,769,021

[45] Oct. 30, 1973

[54] LIGHT-SENSITIVE DIAZOTYPE COPYING MATERIAL

[75] Inven Tadashi Saito, Kanagawa; Kiyoshi Sakai, Tokyo, both of Japan

[73] Assignee: **Kabushiki Kaisha Ricoh**, Tokyo, Japan

[22] Filed: **Feb. 12, 1971**

[21] Appl. No.: **115,057**

## Related U.S. Application Data

[63] Continuation-in-part of Ser. No. 659,609, Aug. 10, 1967, abandoned.

## Foreign Application Priority Data

Aug. 26, 1966 Japan..... 41/55819  
Nov. 29, 1966 Japan..... 41/77761  
Nov. 29, 1966 Japan..... 41/77762

[52] U.S. Cl..... **96/91 R, 260/141, 96/49**

[51] Int. Cl..... **G03c 1/54**

[58] Field of Search..... **96/91.75, 49; 260/141, 142**

## References Cited

### UNITED STATES PATENTS

3,272,630 9/1966 Rauhut et al. .... 96/91 X  
3,379,531 4/1968 Mizianty et al. .... 96/91

|           |         |                     |       |
|-----------|---------|---------------------|-------|
| 3,432,301 | 3/1969  | Rauhut et al. ....  | 96/91 |
| 3,281,246 | 10/1966 | Rauhut et al. ....  | 96/91 |
| 3,462,271 | 8/1969  | Rauhut et al. ....  | 96/91 |
| 59,551    | 8/1969  | Rauhut et al. ....  | 96/91 |
| 42,652    | 5/1969  | Hectors et al. .... | 96/91 |

## FOREIGN PATENTS OR APPLICATIONS

|           |        |                     |         |
|-----------|--------|---------------------|---------|
| 957,838   | 5/1964 | Great Britain ..... | 96/91 R |
| 919,037   | 2/1958 | Great Britain ..... | 96/91 R |
| 867,630   | 5/1961 | Great Britain ..... | 96/91 R |
| 1,110,835 | 4/1968 | Great Britain ..... | 260/141 |

## OTHER PUBLICATIONS

Reproduction Paper News Bulletin, Andrew Paper & Chem. Co. Inc. No. 26, Sept. 1960.

Landau, R., "Fascicles 1a8 (Les diazo)", Distributed by Andrews Papers & Chem. Co. Inc., 1960, p. 30 relied on.

Primary Examiner—Charles L. Bowers, Jr.

Attorney—Woodhams, Blanchard & Flynn

## [57] ABSTRACT

A diazotype copying material having a light-sensitive coating containing a diazonium salt selected from the group consisting of 2,5-disubstituted derivatives of 4-dibenzylamino-benzene diazonium salt exhibits a very high sensitivity to light.

1 Claim, No Drawings

**LIGHT-SENSITIVE DIAZOTYPE COPYING MATERIAL**

**CROSS-REFERENCE TO RELATED APPLICATION**

This application is a continuation-in-part of our co-pending application Ser. No. 659 609, filed Aug. 10, 1967, now abandoned.

**BACKGROUND OF THE INVENTION**

**FIELD OF THE INVENTION**

The present invention relates to a light-sensitive diazotype copying material and more particularly to a highly light-sensitive diazotype copying material whose copying layer contains a novel 4-dibenzylaminobenzene diazonium compound.

**DESCRIPTION OF THE PRIOR ART**

In the field of copying techniques which utilize diazonium compounds, there has been a demand, since the time such techniques were found, for copying materials high in light-sensitivity or, in other words, a demand for diazonium compounds having high sensitivity to light. This demand has been on the increase of late, because fluorescent lamps which are not only less expensive but also smaller in the total radiation energy than mercury lamps have become utilized widely as the light source for diazotype copying. In order to meet this increasing demand, there have been introduced various kinds of derivatives of p-aminobenzene diazonium compounds having relatively high sensitivity to light.

**SUMMARY OF THE INVENTION**

The present invention contemplates the provision of novel p-dibenzylaminobenzene diazonium compounds having a very high sensitivity to light and coupling property, and also contemplates the provision of diazotype copying materials employing such compounds.

Specifically, the present invention contemplates the provision of diazotype copying materials featured in that their light-sensitive copying layers contain at least one of the diazonium compounds which are expressed by the following general formula:



wherein:

R is selected from the group consisting of a hydroxyl radical, an alkoxy or phenyl-substituted alkoxy radical having from one to four carbon atoms in the alkyl chain, a morpholino radical, a pyrrolidino radical, a piperidino radical, a piperazino radical and



wherein R<sub>1</sub> and R<sub>2</sub> are alkyl radicals having from one to four carbon atoms;

Y is selected from the group consisting of hydrogen, an alkyl radical having from one to four carbon

atoms, an alkoxy radical having from one to four carbon atoms, a hydroxyl-substituted alkoxy radical having from one to four carbon atoms, and a morpholino-, pyrrolidino-, piperidino- or piperazino-substituted alkoxy radical having from one to four carbon atoms;

n is an integer between 1 and 4; and X represents an anionic radical.

The diazonium compounds according to the present invention may be applied to one-component copying materials which are developed according to the moist-development method, two-component copying materials which are developed according to the dry-development method and also to three-component copying materials which are developed according to the thermal development method. By the use of these diazonium compounds of the present invention, there are obtained copies of images varying in color such as black and blue, depending on the type of the azo coupling component used. According to the present invention, the light-sensitive copying layer is coated on a support such as paper, precoated paper and plastic foil which is used in ordinary diazotype copying materials. This copying layer may contain an additive such as an anti-yellowing agent and a stabilizer.

The diazonium compounds used in the present invention are prepared, in many cases, in the form of diazonium chloride or double salt of diazonium chloride and metal chloride, and in particular, they are obtained in the form of double salts of diazonium chloride and zinc chloride or double salts of diazonium chloride and cadmium chloride. In the present invention, however, the type of anion which is coupled to the diazonium cation is not critical. Diazonium compounds in the form of, for example, bromides, sulfates and fluoroborates may also be used in the present invention.

With respect to the general formula of the diazonium compounds of the present invention, the preferred alkyl radicals include methyl, ethyl, n-propyl, isopropyl, n-butyl and tert-butyl. The preferred alkoxy radicals include methoxy, ethoxy, n-propoxy, iso-propoxy and n-butoxy. The preferred



radicals include N-methylamino, N-ethylamino, N,N-dimethylamino, N,N-diethylamino and N,N-n-propylamino.

As has been stated, the diazonium compounds of the present invention may be applied to one-component, two-component and three-component copying materials. The diazonium compounds show an increased coupling velocity and such compounds are particularly suitable for both one-component and two-component copying materials.

Hereunder are enumerated typical diazonium compounds which are used in the present invention. It should be understood, however, that the diazonium compounds which are usable in the present invention are not restricted to these compounds alone.

Formula 1



Formula 2



Formula 3



Formula 4



Formula 5



Formula 6



Formula 7



Formula 8



Formula 9



Formula 10



5

(131~136° C.)  
[405~410 mμ]

Formula 11



15

(135~140° C.)  
[405~410 mμ]

NOTE: (Decomposition point), [ultraviolet absorption].

Methods for preparing selected ones of the above-referenced diazonium compounds are as follows:

20

## FORMULA 1

Seventy grams of 5-( $\beta$ -hydroxy) ethoxyaniline and 82 g of sodium acetate were dissolved in 50 ml of water. While holding the temperature of this solution between 90°C. and 100°C., 127 g of benzyl chloride were added, in drops, to the solution while stirring. After the mixture was left to react for about five hours, the supernatant oil layer was removed and distilled under a reduced pressure of 1 mmHg. As a result, 85 g of distillate boiling between 240°C. and 255°C. were obtained (This substance had a melting point between 66.5°C. and 67.5°C.). This distillate was coupled to a diazonium compound of p-nitroaniline to produce a dyestuff, with the yield being 57 g (The resulting substance has a melting point between 202°C. and 204°C.). This dyestuff was then reduced with hydrogen gas to an amino compound. This latter compound was reacted with acetic anhydride to cause N,N'-diacetyl-p-diaminobenzene to separate out. The obtained acetyl compound was subjected to hydrolysis, followed by diazotization in a known manner. The resulting diazonium compound was salted out with zinc chloride. Thus 15 g of 4-dibenzylamino-5-( $\beta$ -hydroxy) ethoxy benzene diazonium chloride, zinc chloride double salt which was yellow in color were obtained. This double salt had a decomposition point between 123°C. and 125°C., and had a peak of ultraviolet absorption at 410 m $\mu$ .

50

## FORMULA 2

One hundred twenty-one grams of 5-( $\beta$ -benzyloxy) ethoxy aniline and 82 g of sodium acetate were dissolved in 50 ml of water. While holding the temperature of this solution between 90°C. and 100°C., 127 g of benzyl chloride were added, in drops, to the solution while stirring. After the mixture was left to react for about six hours, the supernatant oil layer was removed and dissolved in 400 ml of toluene. The resulting solution was subjected to washing with water two or three times and to dehydration with anhydrous sodium sulfate. Then, hydrogen chloride gas was introduced into the solution, 115 g of chloride were separated from the solution (This chloride had a melting point between 210°C. and 212°C.). This chloride was dissolved in acetic acid and coupled, in the presence of sodium chloride, to a diazonium compound of p-nitroaniline. The

resulting coupled compound was neutralized with additional sodium acetate, thereby producing a dyestuff, with the yield being 106 g (The resulting substance had a melting point between 210°C. and 212°C.). This dyestuff was then reduced with hydrogen gas to an amino compound. This latter compound was reacted with acetic anhydride to cause N,N'-diacetyl-p-diaminobenzene to separate out. The obtained acetyl compound was subjected to hydrolysis, followed by diazotization by known manner, and salted out by zinc chloride. Thus 18 g of 4-dibenzylamino-5-( $\beta$ -benzyloxy)ethoxybenzene diazonium chloride, zinc chloride double salt which was yellow in color were obtained. This double salt had a decomposition point between 99°C. and 102°C. and a peak of ultraviolet absorption within the range of from 405 m $\mu$  to 410 m $\mu$ .

## FORMULA 4

Eighty-two grams of 2-methyl-5-( $\beta$ -hydroxy)ethoxyaniline and 82 g of sodium acetate were dissolved in 50 ml of water. While holding the temperature of this solution between 90°C. and 100°C., 127 g of benzyl chloride were added, in drops, to the solution while stirring. After the mixture was left to react for about 7 hours, the supernatant oil layer was removed and distilled under a reduced pressure of 1 mmHg. As a result, 98 g of distillate boiling between 243°C. and 248°C. were obtained. This distillate was coupled to a diazonium compound of p-nitroaniline to produce a dyestuff, with the yield being 68 g (The resulting substance had a melting point between 197°C. and 199°C.). This dyestuff was then reduced with hydrogen gas to an amino compound. This latter compound was reacted with acetic anhydride to cause N,N'-diacetyl-p-diaminobenzene to separate out. The obtained acetyl compound was subjected to hydrolysis, followed by diazotization by known manner, and was salted out by zinc chloride. Thus 18 g of 4-dibenzylamino-2-methyl-5-( $\beta$ -hydroxy)ethoxybenzene diazonium chloride, zinc chloride double salt which was yellow in color were obtained. This double salt had a decomposition point between 124°C. and 129°C., and had a peak of ultraviolet absorption within the range of from 410 m $\mu$  to 415 m $\mu$ .

## FORMULA 5

One hundred and five grams of 2-methyl-5-( $\beta$ -pyrrolidino)ethoxyaniline and 82 g of sodium acetate were dissolved in 50 ml of water. While holding the temperature of this solution between 90°C. and 100°C., 127 g of benzyl chloride were added, in drops, to the solution while stirring. After the mixture was left to react for about six hours, the supernatant oil layer was removed and dissolved in 400 ml of toluene. The resulting solution was subjected to washing with water two or three times and to dehydration with anhydrous sodium sulfate. Then, hydrogen chloride gas was introduced into the solution and 112 g of chloride were separated from the solution (This substance had a melting point between 178°C. and 182°C.). This chloride was dissolved in acetic acid and coupled, in the presence of sodium chloride, with a diazonium compound of p-nitroaniline to produce a dyestuff, with the yield being 105 g (The resulting substance had a melting point between 207°C. and 209°C.). This dyestuff was then reduced with hydrogen gas to an amino compound. This latter compound was reacted with acetic anhydride to cause N,N'-diacetyl-p-diaminobenzene to separate out.

The obtained acetyl compound was subjected to hydrolysis, followed by diazotization by known manner, and salted out by zinc chloride. Thus 28 g of 4-dibenzylamino-2-methyl-5-( $\beta$ -pyrrolidino)ethoxybenzene diazonium chloride, zinc chloride double salt which was yellow in color were obtained. This double salt has a decomposition point between 128°C. and 132°C. and a peak of ultraviolet absorption within the range of 410 m $\mu$  to 415 m $\mu$ .

## FORMULA 8

One hundred eleven grams of 2-methyl-5-( $\beta$ -morpholino)ethoxyaniline and 82 g of sodium acetate were dissolved in 50 ml of water. While maintaining the temperature of this solution between 90°C. and 100°C., 127 g of benzyl chloride were added, in drops, to the solution while stirring. After the mixture was left to react for about six hours, the supernatant oil layer was removed and dissolved in 400 ml of toluene. The resulting solution was subjected to washing with water two or three times and to dehydration with anhydrous sodium sulfate. Then, hydrogen chloride gas was introduced into the solution and 121 g of chloride were separated from the solution (This substance had a melting point between 185°C. and 187°C.). This chloride was dissolved in acetic acid and coupled, in the presence of sodium acetate, with a diazonium compound of p-nitroaniline to produce a dyestuff, with the yield being 112 g (The resulting substance had a melting point between 215°C. and 218°C.). This dyestuff was then reduced with hydrogen gas to an amino compound. This latter compound was reacted with acetic anhydride to cause N,N'-diacetyl-p-diaminobenzene to separate out. The obtained acetyl compound was subjected to hydrolysis, followed by diazotization by known manner, and salted out by zinc chloride. Thus 28 g of 4-dibenzylamino-2-methyl-5-( $\beta$ -morpholino)ethoxybenzene diazonium chloride, zinc chloride double salt which was yellow in color were obtained. This double salt had a decomposition point between 118°C. and 120°C. and a peak of ultraviolet absorption within the range of 400 m $\mu$  to 405 m $\mu$ .

## FORMULA 10

One hundred grams of 2,5-( $\beta$ -hydroxy)ethoxyaniline and 82 g of sodium acetate were dissolved in 50 ml of water. While holding the temperature of this solution between 90°C. and 100°C., 127 g of benzyl chloride were added, in drops, to the solution while stirring. After the mixture was left to react for about 5 hours, the supernatant oil layer was removed and distilled under a reduced pressure of 1 mmHg. As a result, 95 g of distillate boiling between 257°C. and 261°C. were obtained. This distillate was coupled to a diazonium compound of p-nitroaniline to produce a dyestuff, with the yield being 75 g (The resulting substance had a melting point between 208°C. and 210°C.). This dyestuff was then reduced with hydrogen gas to an amino compound. This latter compound was reacted with acetic anhydride to cause N,N'-diacetyl-p-diaminobenzene to separate out. The obtained acetyl compound was subjected to hydrolysis, followed by diazotization by known manner, and salted out by zinc chloride. Thus 32 g of 4-dibenzylamino-2,5-( $\beta$ -hydroxy)ethoxybenzene diazonium chloride, zinc chloride double salt which was yellow in color were ob-

tained. This double salt had a decomposition point between 130°C. and 136°C., and had a peak of ultraviolet absorption within the range of from 405 m $\mu$  to 410 m $\mu$ .

#### FORMULA 11

One hundred seventy-six grams of 2,5-di( $\beta$ -morpholino) ethoxyaniline and 82 g of sodium acetate were dissolved in 50 ml of water. While maintaining the temperature of this solution between 90°C. and 100°C., 127 g of benzyl chloride were added, in drops, to the solution while stirring. After the mixture was left to react for about six hours, the supernatant oil layer was removed and dissolved in 400 ml of toluene. The resulting solution was subjected to washing with water two or three times and to dehydration with anhydrous sodium sulfate. Then, hydrogen chloride gas was introduced into the solution and 131 g of chloride were separated from the solution (This substance had a melting point between 217°C. and 219°C.). This chloride was dissolved in acetic acid and coupled, in the presence of sodium chloride, to a diazonium compound of p-nitroaniline. The resulting coupled compound was neutralized with sodium acetate, thereby producing a dyestuff, with the yield being 125 g (The resulting substance had a melting point between 231°C. and 233°C.). This dyestuff was then reduced with hydrogen gas to an amino compound. This latter compound was reacted with acetic anhydride to cause N,N'-diacetyl-p-diaminobenzene to separate out. The obtained acetyl compound was subjected to hydrolysis, followed by diazotization by known manner, and salted out by zinc chloride. Thus 51 g of 4-dibenzylamino-2,5-( $\beta$ -morpholino) ethoxybenzene diazonium chloride, zinc chloride double salt which was yellow in color were obtained. This double salt had a decomposition point between 135°C. and 140°C. and a peak of ultraviolet absorption within the range of 405 m $\mu$  to 410 m $\mu$ .

#### DESCRIPTION OF THE PREFERRED EMBODIMENTS

##### EXAMPLE 1

A white support for use in diazotype copying materials was precoated with an emulsion consisting of finely granular silica and vinyl acetate. Onto this precoated support was applied a solution having the following composition:

4-dibenzylamino-5-( $\beta$ -hydroxy) ethoxy benzene diazonium chloride, zinc chloride double salt (refer to Formula 1) — 1.3 g  
 Tartaric acid — 0.4 g  
 Boric acid — 0.1 g  
 Water — 100 ml  
 and the sheet was dried.

An original was placed on the light-sensitive copying layer thus obtained and was exposed to light by the use of an illuminating apparatus employing a fluorescent lamp to form a latent image on the layer. This exposure was completed in a very short length of time. The copying layer carrying the latent image was developed in a solution having the following composition:

Thiourea — 1.5 g  
 Phloroglucin — 0.4 g  
 Benzoic acid — 0.25 g

Sodium benzoate — 1.5 g  
 Sodium phosphate — 1.5 g  
 Water — 100 ml

5 The developing solution had a pH of about 5.9. The development was carried out rapidly, and the obtained copy had an image of black in color. The half tone areas of the image obtained were consistent in color with the maximum density areas of this reproduced image.

#### EXAMPLE 2

A support for use in ordinary diazotype light-sensitive copying materials was coated with a sensitizing solution of the following composition:

4-dibenzylamino-2,5-( $\beta$ -hydroxy) ethoxybenzene diazonium chloride, zinc chloride double salt (Refer to Formula 10) — 1.5 g

20 Tartaric acid — 6.0 g

Boric acid — 1.0 g

Acetic acid — 2.0 g

Water — 100.0 g

Caffeine — 0.5 g

25 Methyl cellulose — 0.08 g

Iso-propanol — 3.0 g

2-hydroxy naphthalene-3-carboxylic acid-di-(2'-hydroxyethyl) amide — 3.0 g

and the paper was dried. The coated layer was exposed to light in a manner similar to that described in Example 1 and the resulting layer was brought into contact with an ammonia gas having a high ammonia concentration to develop the image. The developed copy showed a deep blue image.

35 In case the development was performed by the use of an alkaline aqueous solution composed of:

Potassium metaborate — 3 g

Potassium carbonate — 2 g

Water — 100 g

40 in lieu of the aforementioned ammonia gas, a similar, satisfactory copy was obtained.

#### EXAMPLE 3

A solution consisting of:

Ethyleneglycol monomethylether — 20 g

Formic acid — 3 g

Water — 35 g

Iso-propanol — 40 g

Citric acid — 3 g

Cresyl glutaric acid — 2 g

4-dibenzylamino-2-methyl-5-( $\beta$ -ethoxy) ethoxy benzene diazonium compound, zinc chloride double salt (Refer to Formula 6) — 4 g

55 was applied to an acetyl cellulose sheet and was dried. Development was conducted with an ammonia gas in a manner similar to that of Example 2, and a copy yellow in color was obtained. This copy could be used as a good intermediate original since it has a property to

60 intensively absorb ultraviolet rays and the rays locating in the regions near thereof.

We claim:

65 1. A light-sensitive copying material for the diazotype process comprising a support and a photosensitive layer coated on said support, said layer comprising a diazonium compound having the formula:

9



wherein:

R is selected from the group consisting of hydroxyl, alkoxy having from one to four carbon atoms, a group of the formula

10



in which R3 is alkylene having from one to four carbon atoms, aryloxy,



5 wherein R1 and R2 are alkyls having from one to four carbon atoms;

Y is selected from the group consisting of hydrogen, alkyl having from one to four carbon atoms, alkoxy having from one to four carbon atoms, and a group of the formula —OR4Z in which R4 is alkylene having from one to four carbon atoms and Z is —OH,



15 n is an integer between one and four; and X represents an anionic radical.

\* \* \* \* \*

20

25

30

35

40

45

50

55

60

65

10

